

June 11, 1935.

H. DREYFUS

2,004,272

PRODUCTION OF ARTIFICIAL PRODUCTS

Filed July 22, 1931

FIG. 1



FIG. 2



INVENTOR

HENRY DREYFUS

BY *J. S. & C. Weisweiler*  
ATTORNEYS

## UNITED STATES PATENT OFFICE

2,004,272

## PRODUCTION OF ARTIFICIAL PRODUCTS

Henry Dreyfus, London, England

Application July 22, 1931, Serial No. 552,545  
In Great Britain July 30, 1930

10 Claims. (Cl. 18—54)

This invention relates to the production of filaments, yarns, threads, ribbons, films and other products from viscose or other solutions of cellulose or of cellulose derivatives.

5 In my prior U. S. application S. No. 488,830 filed 15th October, 1930 I have described the production of filaments, threads, ribbons and other products from solutions of viscose by coagulating the viscose in the form of a metallic cellulose xanthate and thereafter treating the formed products to regenerate the cellulose. The regeneration of the cellulose could, for instance, be effected by treating the formed products with strong acids, for instance with strong mineral acids, organo mineral acids or acid esters thereof. By this means products were obtainable of fine denier or small cross-section and of high strength.

20 I have now found a further means by which products of very fine denier or small cross-section and also of high strength may be obtained from solutions of viscose and in addition the process of the invention is applicable to the production of filaments or other products from cuprammonium solutions of cellulose or other solutions of cellulose or cellulose derivatives. According to the present invention the solution of cellulose or of a cellulose derivative is extruded into a medium so that little or no elimination 25 of the solvent takes place from the viscose or other solution or at least after passage through the medium the viscose or other product is still liquid or substantially liquid.

30 Preferably the viscose, cuprammonium cellulose or other solution of cellulose or cellulose derivative adapted to yield products of regenerated cellulose is extruded into a liquid which is a non-solvent for the cellulose or for the cellulose derivative and is a non-solvent for the solvent 35 of the spinning solution, for instance water in the case of viscose. Hydrocarbons or halogenated hydrocarbons in the case of viscose or other aqueous solutions of cellulose or of cellulose derivatives are most convenient, since they are 40 substantially non-miscible with water.

45 The halogenated hydrocarbon or other liquid may, if desired, have a specific gravity sufficient to enable the same to rise or fall through the liquid in question. Thus in the case of benzene or other comparatively light hydrocarbons or liquids the nozzle may be directed vertically downwards or downwards at an angle so that the extruded filaments or other products sink or are drawn downwards through the bath of benzene or other light liquid. The specific gravity of the viscose or other spinning solution may itself be adjusted, if desired, as for example by adjusting its concentration or by means of additions made thereto with the object of increasing the specific gravity. As an alternative a liquid

which is heavier than the viscose or other spinning solution may be used, and the viscose or other spinning solution extruded vertically upwards or upwards at an angle into the heavy liquid, and the filaments or other products being drawn off or allowed to rise through the liquid.

5 For convenience of starting up it is preferable however not to rely altogether upon difference in gravity of the spinning solution and the liquid into which it is spun. Starting up may, for example, be effected by spinning initially into a bath adapted to coagulate the cellulose solution, and the bath characteristic of the present invention may be thereafter introduced so 10 that the filaments or other products are already being drawn from the nozzle before the introduction of the said bath.

15 The invention also includes a process in which some elimination of the solvent of the spinning 20 solution takes place in the preliminary stage of the formation of the products described above. For instance in the case of viscose or other aqueous spinning solutions the liquid may be such that it dissolves out a proportion of the 25 water used as solvent in the spinning solution. For this purpose liquids which themselves have a small solvent power for water may be used, or alternatively the hydrocarbons, halogenated hydrocarbons or other water repellent liquids referred to above may be mixed with alcohol, acetic acid, formic acid, lactic acid or other liquids which are adapted to confer thereon a small 30 solvent power for water, and which are at the same time non-solvents for the cellulose xanthate or other base contained in the spinning solution. The amount of water thus abstracted from the filaments or other products should not however be sufficient to prevent their being liquid or substantially liquid on the completion of 35 this preliminary stage of their formation. The length of preliminary bath of hydrocarbon, halogenated hydrocarbon or other suitable liquid in which the filaments or other products are formed may vary very widely. It depends 40 upon the amount of "draw-down", if any, which is applied and on the viscosity of the spinning solution. In most cases a length up to a few inches suffices to produce 45 the advantages of the present invention.

50 The filaments or other products, which may, as described above, be substantially of the same composition as that of the original spinning solution or only have comparatively small amounts of water abstracted therefrom so that they are 55 still liquid, may be coagulated by any convenient method. The coagulation may be such as to effect a simultaneous conversion of the viscose, cuprammonium cellulose or the like into cellulose, as is the case in the art as practised today.

or alternatively the viscose may be coagulated in the form of a metallic or ammonium cellulose xanthate and subsequently treated to regenerate the cellulose. The regeneration of the cellulose, whether carried out simultaneously with or subsequent to coagulation, is preferably effected by means of strong mineral acids or acid esters thereof or by means of sulphonic acids or other organo mineral acids (compare my prior 5 U. S. application S. No. 450,872 filed 8th May, 1930), or alternatively the products in which the cellulose has already been regenerated may be treated subsequently with the strong mineral acids or acid esters or organo mineral acids, 10 preferably continuously with their production.

I have found that by extruding the spinning solution in such a way that none or only a definite proportion of the solvent is abstracted therefrom very fine filament deniers or products 15 of small cross-section are obtainable. At the same time the products have a considerable strength. The invention is however not limited to products of fine denier or small cross-section, since it presents advantages in the manufacture 20 of comparatively large products, such as may be used as artificial horsehair, bristles or the like, products being produced showing high strength as before and also considerable extensibility.

With regard to the details of effecting the 25 preliminary formation of the filaments in a body of liquid and subsequently coagulating the same, I would say that it is convenient to employ the non-solvent liquid contiguous with the coagulating bath proper. Thus for instance benzene or other light hydrocarbon or liquid 30 may be floated on the top of the coagulating bath, the filaments sinking or being drawn through the layer of benzene or like liquid into the coagulating bath wherein they may be coagulated either in the form of cellulose itself or as xanthate and then carried round suitable 35 guides and finally out of the bath. For instance any ordinary tank or other device customarily employed to contain the coagulating liquid may be provided with a partition across the full width of the container but not reaching 40 to the bottom thereof; the container may be partially filled with the coagulating liquid proper at least as far up as the bottom of the partition and then the benzene or other light liquid may 45 be poured into one side only of the partition. The spinning nozzle may then be immersed in the benzene or other light liquid, the filaments or other products carried down into the coagulating 50 liquid, underneath the partition and finally out of the bath. As an alternative in the case of employing as the special liquid for use according to the present invention a comparatively 55 heavy liquid, such as tetrachlorethane, hexachlorethane or other heavy halogenated hydrocarbon, the container may be partially filled with the heavy liquid and the coagulating bath proper poured in so as to form a layer on the top. In this case the spinning nozzle may be 60 immersed at the bottom of the bath and the filaments or other products drawn up through the two layers of liquid.

The coagulating liquid used according to the 65 present invention may consist, in the case of viscose, of comparatively dilute mineral acids, for example sulphuric acid of 5 to 15 or 20% strength, for preference mixed with sodium bisulphate or other salts and/or having additions of glucose or other sugars or like substances, or in the case of cuprammonium solutions of cel-

lulose may consist of relatively dilute caustic soda or other suitable alkaline coagulating liquids. The filaments thus coagulated and regenerated may then be treated with a strong mineral acid or other agent adapted to exert a solvent, 5 softening or incipient solvent action thereon. Such solvent action may be allowed to develop on the filaments or other products by a concentration of the mineral acid or other reagent employed in the coagulating bath itself.

10

Preferably, however, the coagulation and regeneration are effected directly by means of a strong mineral acid or organo mineral acid or a mineral acid ester.

The accompanying drawing illustrates two 15 forms of apparatus suitable for carrying out the process of the present invention, but it is to be clearly understood that the invention is in no way limited to the use of such apparatus.

Referring to Figure 1, a coagulating vessel 3 20 is provided with a partition 4 extending across the full width thereof but not reaching to the bottom of the bath. A bundle of filaments 5 extruded from a jet 6 is led under the partition by means of guides 7 and 8, then round a guide 9 to a draw-roller 10. From the roller it proceeds to a suitable winding or twisting and winding device, e. g. a bobbin 11 which may rotate in a washing liquid contained in a vessel 12. For convenience in starting up, the partition 4 is provided 25 removable, being inserted only after the thread has been led round the thread guides 7, 8 and 9 to the feed roller 10. In carrying out the process with such an apparatus spinning is started up with a coagulating 30 liquid in the customary manner, the bundle of filaments being carried round the guides to the roller 10. After spinning has been begun a medium lighter than the coagulating liquid is run into the compartment of the bath containing 35 the spinning nozzle, until the interfacial surface indicated by line 13' is suitably below the level of the nozzle so that the filaments leave that medium while still in a substantially liquid state. This point in the process is represented in the figure by the passage of the filaments through the lighter medium 13 until they 40 reach the coagulant 14.

30

45

50

Referring to Figure 2, a spinning vessel 15 is provided with a spinning nozzle 16 connected with a candle filter 17 pivoted at 18, the spinning nozzle being adapted to spin upwardly. The filaments 5 produced are conducted round the feed roller 19, to a thread guide 20, through a bath 21 containing a softening liquid, and thence round the roller 22 to a bobbin or other suitable winding device 23, the said bobbin being rotated in running water or sprayed with water from a suitable device 24. This particular form of apparatus is suitable for carrying out the 55 process in which the coagulating liquid 26 is lighter than the medium 27 from which the filaments are removed in substantially liquid form. The latter liquid is run into the spinning bath by means of the tube 25 after spinning 60 has been started up with a normal coagulating bath, forming an interfacial surface 26' above the spinning nozzle.

65

70

The following examples illustrate the invention, but they are not to be considered as limiting it in any way:

#### Example 1

A coagulating vessel is provided with a partition extending across the full width thereof, but 75

not reaching to the bottom of the bath. Beneath the partition a thread guide is arranged adapted to lead the filaments from one compartment of the bath to the other compartment. 5 In one compartment is arranged a spinning nozzle adapted to spin downwards, the height of the spinning nozzle being conveniently 3 or 4 inches above the bottom of the partition. The bath is filled to a point above the spinning nozzle 10 with a 65-80% aqueous solution of sulphuric acid or a 60-70% solution of benzene sulphonic acid. Spinning is then started up with a viscose solution in the customary manner, the filaments being carried round the thread guide and out 15 of the bath through the compartment not containing the spinning nozzle. The thread is carried round a feed roller adapted to exert the required tension and thence to a centrifugal spinning box or a bobbin or other winding or 20 winding and twisting device. Conveniently while being fed into the spinning box or while being wound on the bobbin the strong acid is removed from the filaments by winding. A bobbin may, for instance, be rotated in running 25 water. After spinning has begun benzene is run into the compartment of the coagulating bath containing the spinning nozzle until its level reaches a point 1 to 2 inches below the spinning nozzle. Spinning is thereafter continued. The speed of the feed roller may be increased after the introduction of the benzene, so as to obtain filaments of unusually fine 30 denier.

*Example 2*

35 A spinning vessel provided with a spinning nozzle adapted to spin upwardly is filled with an aqueous solution containing 10% of sulphuric acid, 1% of ammonium sulphate, 15% of sodium sulphate and 10% of glucose. Spinning is started up with a viscose solution, preferably 40 obtained from an unmatured alkali cellulose or from an alkali cellulose which has been matured for a comparatively short time, and the formed 45 filaments are carried round a feed roller and thence into a bath consisting of a 60% aqueous solution of sulphoacetic acid. The yarn is carried out of the coagulating bath and wound on a bobbin rotating in running water or sprayed 50 with water. After starting up, tetrachlorethane is run into the bottom of the spinning bath, for example by means of a suitable tube or pipe reaching to the bottom, until it covers the spinning nozzle to the extent of 1 to 2 inches. Spinning is thereafter conducted as described in 55 Example 1.

The term "cellulosic solution", as used hereinafter in the claims, is to be understood as meaning solutions of cellulose or of derivatives thereof which are relatively unstable and capable of ready regeneration, e. g. viscose and the term does not include solutions of organic esters or ethers of cellulose, which are relatively 60 stable.

65 What I claim and desire to secure by Letters Patent is:—

70 1. Process for the manufacture of filaments, yarns, threads, ribbons, films and like extruded products from aqueous cellulosic solutions, comprising extruding the said solutions into liquids which are water-repellent, continuously removing the products from said liquid whilst they are still liquid and thereafter setting the said 75 products.

2. Process for the manufacture of filaments, 5 yarns, threads, ribbons, films and like extruded products from aqueous cellulosic solutions, comprising extruding the said solutions into a liquid medium comprising hydrocarbons which is a non-solvent for the constituents of the solutions, continuously removing the products from said medium whilst they are still liquid, and thereafter setting the said products.

3. Process for the manufacture of filaments, 10 yarns, threads, ribbons, films and like extruded products from aqueous cellulosic solutions, comprising extruding the said solutions into a liquid medium comprising halogenated hydrocarbons which is a non-solvent for the constituents of 15 the solutions, continuously removing the products from said medium whilst they are still liquid, and thereafter setting the said products.

4. Process according to claim 1 wherein the 20 cellulosic solutions are passed through the medium for a comparatively short distance of the order of 1 to 2 inches.

5. Process for the manufacture of filaments, 25 yarns, threads, ribbons, films and like extruded products from solutions of viscose, comprising spinning the said solutions into a liquid medium which is a non-solvent for the constituents of the solutions and continuously removing the same from said medium while the products are still liquid, and thereafter setting the said filaments and regenerating the cellulosic base thereof by treatment in an acid bath.

6. Process according to claim 5 wherein the 35 acid present in the bath is a body selected from the group consisting of strong mineral acids and acid esters thereof and organo mineral acids.

7. Process according to claim 1 wherein the 40 filaments or other products are drawn down to products of low denier or small cross-section prior to completion of the setting.

8. Process for the manufacture of filaments, 45 yarns, threads, ribbons, films and like extruded products from solutions of viscose, which comprises extruding the said solutions into a liquid medium which is a non-solvent for the constituents of the solutions and continuously removing the products from said medium while they are still liquid, and thereafter setting the products and regenerating the cellulosic base thereof, the 50 formed products being subjected to a stretching operation prior to completion of the setting.

9. Process for the manufacture of filaments, 55 yarns, threads, ribbons, films and like extruded products from aqueous cellulosic solutions, which comprises extruding the said solutions into liquids which are water-repellent, continuously removing the products from said liquids while they are still liquid and thereafter setting the products, the formed products being submitted to a stretching operation prior to completion of the setting.

10. Process for the manufacture of filaments, 60 yarns, threads, ribbons, films and like extruded products from solutions of viscose, which comprises extruding the said solutions into a liquid medium which is a non-solvent for the constituents of the solutions and continuously removing the products from said medium while they are still liquid, and thereafter setting the products 70 and regenerating the cellulosic base thereof, the formed products being submitted to a stretching operation prior to regeneration.